

## UNITED STATES PATENT OFFICE.

GILBERT JOHNSON WILDRIDGE, OF CALDERCRUIX, SCOTLAND.

## MATERIAL FOR MATRICES.

SPECIFICATION forming part of Letters Patent No. 744,889, dated November 24, 1903.

Application filed June 8, 1903. Serial No. 160,662. (No specimens.)

*To all whom it may concern:*

Be it known that I, GILBERT JOHNSON WILDRIDGE, managing director of Robert Craig and Sons, Limited, paper manufacturers, a subject 5 of the King of Great Britain and Ireland, residing at Caldercruix Mills, Caldercruix, in the county of Lanark, Scotland, have invented certain new and useful Improvements in Material for Matrices, of which the following 10 is a specification.

This invention has for its object to produce improved materials to be used in making matrices for use, either wet or dry, in casting for printing and other purposes and technically 15 known as "flongs." Hitherto such materials or flongs have most generally been prepared by pasting together or otherwise building up by hand sheets of paper or a sheet or sheets of paper with other materials so as to constitute 20 a matrix-making material or flong.

The object of this invention is to make in a more efficient and economical manner than hitherto a matrix-making material or flong of an improved character and consisting of a 25 stiff backing, a bed or intermediate layer of a plastic character, and a face made as hereinafter described, which flong will receive clear and sharp impressions from the type or the like without the material of the face of 30 the matrix being broken by the type or the like or destroyed by the hot metal which is cast in the matrix, so that the matrix can be used for a number of castings, great saving in time in preparing the matrix for casting 35 being effected by the use of such flongs.

According to my invention the face of the matrix-making material or flong (which face comes into contact with the type or the like in forming the matrix and with the hot metal 40 in casting) is made of a mixture of pulped material having pliable and tough fibers with a substance which is resistant to the action of heat, and preferably also with a substance which will prevent the cast metal adhering to 45 the face of the matrix and help to produce a glossy finish on the face of the matrix. It is preferred to use no size in making this face, and the fibrous material used should be so milled or treated in the pulper that the fibers 50 are as pliable as possible. I have found that flax is best suited for this purpose, that silicate of magnesia is suitable for use as the

heat-resisting substance, and that borax is suitable for use as the substance for preventing adherence of the casting to the face of the matrix and for helping to produce a glossy finish on the said face. A good mixture for the said face consists of one hundred parts, by weight, of flax, twenty-five parts, by weight, of silicate of magnesia, and three parts, by 60 weight, of borax; but I do not limit myself to these proportions. A suitable material for the bed or intermediate layer is cotton, with or without kaolin or the like and without size. The backing layer may be made of any suitable 65 paper-making materials and may have size in it, together with starch or kaolin, or both, if desired.

The layers of pulped materials are brought together on paper-making machinery, which 70 may be done as follows: The pulps for the several layers—namely, the face layer, the back layer, and the bed or intermediate layer—are contained in separate vats, from which the several layers are produced, and these layers 75 are brought together at any suitable part of a paper-making machine while they are in a condition such that they adhere together and form a composite material of the character aforesaid. For example, one layer—say the 80 layer for the face—may be brought to the combining place on an ordinary Fourdrinier-machine wire, while the other layers may each be formed by perforated or reticulated (wire-gauze) cylinders rotating in the respective 85 vats containing the pulps for making these layers and be taken up successively by a felt, which conveys the layers of pulp to the part of the paper-making machine where they meet the layer from the machine-wire, so that this 90 layer forms, say, one outer layer, the backing another outer layer, the bed or intermediate layer being between the said two outer layers, or the one layer—say the backing—may be formed on the wire of a Fourdrinier paper-making machine, and the other layers—say 95 the intermediate and face layers—may be formed on perforated or reticulated cylinders, or all the layers may be formed on perforated or reticulated cylinders, or these cylinders 100 may be dispensed with and all the layers be formed upon a series of ordinary paper-making-machine wires, such as are used in Fourdrinier paper-making machines. If desired,

the backing layer may be omitted and a backing material be applied after the other two layers have been combined on the machine. The combined layers are passed over a heated metal cylinder of large diameter and with a highly-polished periphery, the face layer being pressed against this periphery and remaining in contact therewith for a time long enough to sufficiently dry the material, the hot periphery of the cylinder imparting to the face layer a smooth glazed finish, which is necessary for producing a smooth glossy face upon the type or the like on the castings taken from the matrix.

15 Although I mention only three principal layers in this specification and in the claims, each principal layer may of course be composed of two or more constituent layers, these constituent layers of each of the principal 25 layers being of the same character as each other or somewhat varying in character, provided that the main characteristics of the several principal layers be retained.

Having now particularly described and ascertained the nature of this invention and in what manner the same is to be performed, I declare that what I claim is—

1. A material, or "flong," for making matrices for use in casting; the said material, or 30 "flong," consisting of the combination, with a stiff backing layer, and a bed, or intermediate, layer, of a face layer consisting of a mixture of pliable fibers and a substance, such as silicate of magnesia, which is resist-

35 ant to the action of heat.

2. A material, or "flong," for making matrices for use in casting; the said material, or

"flong," consisting of the combination, with a backing layer, and a bed, or intermediate, layer, of a face layer consisting of a mixture 40 of pliable fibers and a substance, such as silicate of magnesia, which is resistant to the action of heat, and of a substance, such as borax, which will prevent the adherence of the cast metal to the matrix, and help to produce a glossy finish on the face.

3. A material, or "flong," for making matrices for use in casting; the said material, or "flong," consisting of the combination, with a backing layer and a bed, or intermediate, layer, of a face layer composed of flax and 45 silicate of magnesia.

4. A material, or "flong," for making matrices for use in casting; the said material, or "flong," consisting of the combination, with 55 a backing layer and a bed, or intermediate, layer, of a face layer, composed of flax and silicate of magnesia and borax.

5. A material, or "flong," for making matrices for use in casting; the said material, or "flong," having a face layer composed of, or 60 containing, pliable fibers, and silicate of magnesia.

6. A material, or "flong," for making matrices for use in casting; the said material, or "flong," having a face layer composed of, or 65 containing, pliable fibers, silicate of magnesia and borax.

In testimony whereof I affix my signature in presence of two witnesses.

GILBERT JOHNSON WILDRIIDGE.

Witnesses:

GEORGE COBB,  
ROBERT FINDLAY SCOTT.